

Oct. 6, 1942.

M. PIPKIN

2,297,981

METHOD OF FROSTING GLASS ARTICLES

Filed April 7, 1939

Fig. 1.



Fig. 2.



Fig. 3.



Fig. 4.



Inventor:  
Marvin Pipkin,  
by Harry E. Dunham  
His Attorney.

## UNITED STATES PATENT OFFICE

2,297,981

## METHOD OF FROSTING GLASS ARTICLES

Marvin Pipkin, Cleveland Heights, Ohio, assignor  
to General Electric Company, a corporation of  
New York

Application April 7, 1939, Serial No. 266,601

1 Claim. (Cl. 41—42)

My invention relates in general to a method of frosting the surface of glass articles, and more particularly to a method of frosting the interior surface of electric lamp bulbs. Still more particularly, my invention relates to a glass article having a frosted surface of distinctive structure.

One object of my invention is to provide an electric incandescent lamp bulb with a relatively rough inside frosted surface which will diffuse the light rays from the filament to such an extent as to eliminate images of the filament and so prevent the occurrence of a bright spot of light within the bulb.

Another object of my invention is to provide a novel method for the production of a relatively heavy frost of distinctive structure on the surface of glass articles.

Still another object of my invention is to provide a reflecting electric incandescent lamp of distinctive appearance and structure in which all sharp images of the lighted filament, as well as the intense mirror effect of the reflecting coating, are eliminated.

Further objects and advantages of my invention will appear from the following detailed description of species thereof and from the accompanying drawing, in which:

Fig. 1 is a longitudinal sectional view of a lamp bulb illustrating a step in the production of the inner frosted surface according to my invention; Fig. 2 is an elevation partly in section of the completed lamp bulb comprising my invention; Fig. 3 is an elevation of a modification of the invention in which a portion of the inner bulb surface is covered with a reflecting coating; and Fig. 4 is a fragmentary sectional view, on an enlarged scale, of the bowl portion of the bulb shown in Fig. 2, illustrating the structure of the heavy frosted surface comprising my invention.

Referring to the drawing, a glass bulb such as is employed for electric incandescent lamps is shown at 18. According to the invention, the entire inner surface of the bulb, or only a portion thereof, is provided with a rough or heavy frost of distinctive structure, as indicated at 11 in Fig. 2. This heavy inner frost is formed by the method comprising my invention, as described herein-after.

As shown in Fig. 1, the bulb 18 is first filled with a quantity of small globular acid-resisting material such as lead bird shot 12, the size of which varies, and the bulb placed in an upright position. The shot may be of any desired size, but preferably should not be finer than that commercially known as No. 15 shot. A sufficient

amount of shot is inserted to cover the inner surface area to be provided with the heavy frost according to the invention. In the particular form illustrated in the drawing, the bulb is filled with sufficient lead shot to cover approximately the lower half or bowl only of the bulbous portion of the bulb. An etching solution that will etch the glass, such as 30 per cent hydrofluoric acid, is then poured into the bulb so as to just cover the lead shot 12. This treating solution is allowed to act on the glass of the bulb for a period of from five to ten minutes without any movement or disturbance of the bulb or its contents, so that the lead shot 12 is maintained in fixed relation to the inner bulb surface throughout the etching operation. The etching solution and the lead shot 12 are then poured out simultaneously and the bulb washed out.

As shown in Figs. 2 and 4, the above-described etching process produces a frosted surface of distinctive structure consisting of a myriad of round peaks or protuberances 13 all separated by relatively large, rounded and interconnected valleys or depressions. With such an etched surface, the rays of light emanating from a filament located within the bulbous portion of the bulb are diffused to such an extent as to eliminate any sharp filament images or bright spots within the bulb.

39 In the bulb illustrated in Figs. 1 and 2, in which only the bowl portion is provided with the frosted inner surface according to the invention, it is desirable to provide the remainder of the inner bulb surface with a relatively light frost or etch 35 14 (Fig. 2), such as is employed at present on conventional electric incandescent lamps. This secondary frosting operation is preferably carried out by first covering the heavy frosted surface 11 with a suitable acid-resisting medium, such as paraffine wax, and then treating the remaining exposed inner surface of the bulb with an etching solution in the manner customary for the production of conventional inside frosted lamp bulbs. The wax covering on the heavy frosted surface 11 is then removed in any suitable way, such as by dissolving.

In the modification shown in Fig. 3, the lamp bulb there shown is the same as that shown in Fig. 2 with the exception that the bowl portion, i. e., the portion provided with the heavy inside frosted surface 11, is covered with an inner reflecting coating 15 of aluminum or silver, or any other suitable reflecting material. The result is a reflecting surface having a myriad of relatively small depressions or dimples 16 therein readily

visible to the eye and presenting a pebbled appearance. Such a reflecting surface gives diffusion to the light rays emanating from the filament, thus eliminating all sharp images of the filament. In addition, such a reflecting surface 15 eliminates the intense mirror effect normally characteristic of a bulb provided with a reflecting coating on a plain glass surface.

While I have described my invention in connection with the production of interiorly frosted electric incandescent lamp bulbs, it is obvious that it may be applied equally as well to the outer surface of such bulbs or to the frosting of flat glass surfaces.

What I claim as new and desire to secure by 15 Letters Patent if the United States is:

A method for the production of inside frosted bulbs which comprises partly filling said bulb with a quantity of loose but closely packed relatively small globules of a substantially acid-resistant material, treating the inner bulb surface covered by said acid-resistant material with an etching solution while maintaining said acid-resistant material in fixed relation to said surface, removing said solution and said acid-resistant material from said bulb, washing the treated inner surface of said bulb and entirely covering the said treated surface with a layer of acid-resistant material, treating the remainder of said inner bulb surface with an etching solution, and removing said layer of acid-resistant material.

MARVIN PIPKIN.